

## UNITED STATES PATENT OFFICE

2,394,588

## PHOTOGRAPHIC DEVELOPER

Frederic R. Bean, Rochester, N. Y., assignor to  
Eastman Kodak Company, Rochester, N. Y., a  
corporation of New Jersey

No Drawing. Application December 8, 1943,  
Serial No. 513,487

5 Claims.

(Cl. 95—88)

This invention relates to photographic developers, and more particularly to developers in which the usual alkalies are replaced by a compound new for the purpose.

One object of my invention is to provide an air-stable, moisture-resistant alkali for use in photographic developers. Another object is to provide an alkali which will give, in photographic developers, approximately the same alkalinity and results as sodium hydroxide. Another object is to provide a stable, non-caking, ready-mixed, dry developer powder. Still another object is to provide a stable, non-caking, ready-mixed, single dry developer powder. Other objects will hereinafter appear.

Alkaline developers have been known and used for many years. These developers usually contain developing agents, a so-called preservative, such as sodium sulfite, and an alkali. One of the oldest and most useful alkalies used in photographic developers is sodium hydroxide, otherwise known as caustic soda. The degree of alkalinity which it confers upon a developer has been found to be most suitable for certain purposes. However, sodium hydroxide is deliquescent and corrosive, and for this reason is difficult to handle, weigh, store and package. Moreover, when used in ready-mixed, packaged developer powders, which, because of their convenience and uniformity, are very popular among both amateur and professional photographers, sodium hydroxide is apt to cause caking, discoloration and deterioration of the powder. This renders impracticable the preparation of a single-powder developer containing sodium hydroxide.

I have discovered that a monosodium derivative of a hexahydric alcohol, such as mannitol or sorbitol, is a suitable substance for use in photographic developers in which it is desired to have the alkaline properties of sodium hydroxide without its undesirable properties. As an example of a method by which such a sodium derivative may be prepared, I give the following:

## Example 1

To 45.5 grams of mannitol, heated to about 180° C.—210° C., 10 grams of solid sodium hydroxide was added gradually, with stirring. After the reaction was complete, the reaction mixture was cooled. A hard, glassy solid was formed, which was moisture resistant and remained unchanged on standing exposed to an atmosphere having a relative humidity between 40—45% for weeks. The yield was about 51 grams, the theoretical amount according to the equation:



Greater than molecular quantities of mannitol or sorbitol may be used in the reaction mixture, conferring even higher moisture resistance to the resulting compound.

When sorbitol was used in place of mannitol, in the same quantity and under practically the same conditions, a similar reaction occurred, giving a product closely resembling that obtained with mannitol.

pH measurements indicated that these products were completely hydrolyzed when dissolved in water. When molecularly equivalent quantities of sodium hydroxide and of sodium mannitoxide were dissolved separately in water, they gave the same pH or alkalinity.

Sodium mannitoxide and the corresponding monosodium derivative of sorbitol are stable, moisture resistant compounds which can be weighed, stored and handled with ease. They can be used in place of sodium hydroxide, in molecularly equivalent proportions, in all photographic developer formulae in which sodium hydroxide is used, with the same photographic results. Moreover, they can be used to prepare single-powder developers, since they do not react upon the other dry chemicals present in the powder.

As an example of a single-powder developer containing sodium mannitoxide, I give the following. It will be understood that this example is illustrative only, and that sodium mannitoxide, or the equivalent monosodium derivative of another hexahydric alcohol, such, for instance, as sorbitol, may be substituted for the molecularly equivalent amount of sodium hydroxide in any photographic silver-image developer formula, whether the developer be in dry form or in solution.

## Example 2

|                         | Grams |
|-------------------------|-------|
| Sodium sulfite          | 11.25 |
| 45 Hydroquinone         | 5.62  |
| Sodium mannitoxide      | 30.00 |
| Potassium bromide       | 3.75  |
| Potassium metabisulfite | 5.00  |

For use dissolve in 250 cc. of water.

50 This developer has all ingredients mixed intimately together in a single container and remains stable in dry form, without discoloration. When a single powder was prepared, containing the same ingredients in the same proportions, except that 6.68 g. of sodium hydroxide was sub-

stituted for the 30 g. of sodium mannitoxide, discoloration and deterioration occurred immediately.

If a buffered solution is desired from a single-powder developer in which sodium mannitoxide or other mono-sodium derivative of a hexahydric alcohol is used, boric acid can be added in sufficient quantity to get the buffer effect. 5

What I claim as my invention and desire to be secured by Letters Patent of the United States is: 10

1. A photographic developer containing a developing agent and a monosodium derivative of a hexahydric alcohol as an alkali.
2. A photographic developer containing a de-

veloping agent and a monosodium derivative of manitol as an alkali.

3. A photographic developer containing a developing agent and a monosodium derivative of sorbitol as an alkali.

4. A photographic developer, in dry form, containing a developing agent and a monosodium derivative of a hexahydric alcohol as an alkali.

5. A photographic developer in the form of a single dry powder, containing a developing agent and a monosodium derivative of a hexahydric alcohol as an alkali.

FREDERIC R. BEAN.